

Patented Aug. 7, 1945

2,381,242

# UNITED STATES PATENT OFFICE

2,381,242

## MOLDING SAND AND METHOD OF CONTROLLING FLOWABILITY OF SAME

Robert T. Wood, Cleveland, Ohio, assignor to Aluminum Company of America, Pittsburgh, Pa., a corporation of Pennsylvania

No Drawing. Application November 21, 1941,  
Serial No. 419,852

8 Claims. (Cl. 22—188)

This invention relates to the art of casting metal members in sand molds, and it is more particularly concerned with the provision of a method of controlling, increasing, and maintaining the flowability of used green sands.

In present sand foundry practice, green sands are employed for the casting of a variety of metals, including the light metals aluminum, magnesium, and their alloys. The constituents of such sands vary somewhat, depending on the use to which they are put, but most of them contain a clay bonding material. Sands used for making molds in which magnesium is cast are usually bonded with bentonite and contain certain additional substances to inhibit oxidation of the molten metal. For example, relatively small amounts of various inhibiting agents such as boric acid and sulfur are introduced into the sand. Such substances as glycerine, ethylene glycol, diethylene glycol, or other polyhydric alcohols which are disclosed in U. S. Patent No. 1,868,453 are frequently employed, usually in combination with the boric acid and sulfur. The use of small amounts of certain fluorides that will decompose or vaporize has been proposed as another means of inhibiting oxidation of molten magnesium in sand molds.

It is important that molding sand possess certain desired physical characteristics. It should be relatively strong so that the mold will retain its shape during handling and casting operations. However, while the sand should have the requisite strength, it should not possess this property in such high degree as to be regarded as tough. The sand should also be relatively flowable, that is, take the shape of the pattern easily when the mold is being made. This property of flowability permits the sand, when rammed, to conform to every portion of the pattern, and thus enables the production of castings having sharply defined contours and smooth surfaces.

In ordinary foundry practice, the molding sand is used over and over again, and it is desirable that the sand retain its initial physical properties throughout the period of use. It has been found, however, that with continued usage sands containing bentonite or other similar bonding materials have a tendency to become somewhat tougher and less flowable. Such bonding materials are herein referred to as argillaceous bonding substances. This tendency seems to be more noticeable in magnesium molding sands containing sulfur and other special oxidation inhibiting agents. This seriously interferes with the production of accurate, smooth castings and

makes the ramming of the molds much more difficult. It is not fully understood why this decrease in flowability should occur, but it is thought to relate to the polymerization and colloidal suspension of various constituents in the sand.

It is, therefore, an object of this invention to overcome the foregoing deficiency of used molding sands. More particularly, it is an object to 10 provide a means of restoring the initial flowability of a used molding sand and to control the same throughout the subsequent period of use of the sand. A still further object is to attain such results in molding sands used in the casting of light metals, particularly magnesium.

I have discovered that potassium fluoride, or sodium fluoride, or both, when introduced into tough sand in suitable amount, reduce the toughness and increase the flowability. Through use 20 of these compounds, it is possible not only to attain these results but also to control them throughout the subsequent period of use of the sand. For the purpose of my invention, these fluorides are considered as constituting a group 25 of substances which control the flowability and toughness of molding sands containing bentonite or similar argillaceous bonding material. While either of the fluorides, or mixtures of them, may be employed, I prefer to use potassium fluoride 30 since this material seems to give somewhat superior results.

In general, the type of molding sands to which I propose to add sodium or potassium fluoride may be either natural or synthetic. Synthetic 35 sands generally contain a mixture of about 90 to 95 per cent sharp silica sand and about 2 to 5 per cent bentonite or other similar bonding material, whereas natural molding sands usually contain an even larger per cent of a bonding 40 medium. To either type of sand I add about 0.10 to 2.0 per cent of either sodium fluoride or potassium fluoride, and where a mixture is employed, the total amount should not exceed about 2 per cent nor should the minimum amount of 45 each fluoride be less than 0.1 per cent, though, as stated above, I prefer to employ only potassium fluoride. When this latter substance is employed, it is preferably added within the limits of 0.25 to 0.5 per cent. These figures represent parts 50 by weight of the dry mixture. In addition to the above named substances, a suitable magnesium molding sand will also contain 1 to 2 per cent sulfur, 1 to 2 per cent boric acid, with or 55 without about 1.5 to 2.5 per cent by weight of glycol or other suitable oxidation inhibiting agent.

The sodium and potassium fluoride addition has very little, if any, oxidation inhibiting effect in magnesium molding sands, and therefore cannot be considered as belonging to the group of oxidation inhibitors used in such sands.

It has been noted that with the continued usage of the sand to which sodium or potassium fluoride has been added, some small loss of the added fluoride may occur. In such instances it is very important that the fluoride content of the sand be maintained within the approximate limits indicated above by suitable additions from time to time. The fluorides of sodium and potassium are nevertheless relatively stable substances in comparison with organic compounds or other substances which are added to molding sands, especially magnesium molding sand, that decompose or vaporize and escape from the sand.

Having thus described my invention,

I claim:

1. The method of controlling the flowability of used molding sands containing an argillaceous bonding material which comprises adding thereto, and maintaining therein, from about 0.1 to 2 per cent of at least one fluoride of the group consisting of sodium fluoride and potassium fluoride.

2. The method of controlling the flowability of a used synthetic molding sand containing from about 2 to 5 per cent bentonite, which comprises adding thereto and maintaining therein, from about 0.1 to 2 per cent of at least one fluoride of the group consisting of sodium fluoride and potassium fluoride.

3. The method of improving the flowability of a used magnesium molding sand containing from about 3 to 5 per cent bentonite, 1 to 2 per cent sulfur, and 1 to 2 per cent boric acid, which comprises adding thereto and maintaining therein, from about 0.1 to 2 per cent of at least one fluoride selected from the group consisting of sodium fluoride and potassium fluoride.

4. The method of improving the flowability of a used magnesium molding sand containing from

about 2 to 5 per cent bentonite, 1 to 2 per cent sulfur, 1 to 2 per cent boric acid, and 1.5 to 2.5 per cent of a polyhydric alcohol, which comprises adding thereto and maintaining therein, from about 0.1 to 2 per cent of at least one fluoride selected from the group consisting of sodium fluoride and potassium fluoride.

5. A used molding sand containing an argillaceous bonding material and from about 0.1 to 2 per cent of at least one fluoride selected from the group consisting of potassium fluoride and sodium fluoride, said sand being characterized by a flowability substantially equivalent to that of the original sand prior to use and the addition of said fluoride constituent.

6. A used molding sand for casting magnesium containing about 2 to 5 per cent bentonite, 1 to 2 per cent sulfur, 1 to 2 per cent boric acid, and 0.1 to 2 per cent of at least one fluoride from the group consisting of potassium fluoride and sodium fluoride, said sand being characterized by a flowability substantially equivalent to that of the original sand prior to use and the addition of said fluoride constituent.

7. A used molding sand for casting magnesium containing about 2 to 5 per cent of an argillaceous bonding material, 1 to 2 per cent sulfur, 1 to 2 per cent boric acid, 0.25 to 0.5 per cent potassium fluoride, and about 1.5 to 2.5 per cent of a polyhydric alcohol, said sand being characterized by a flowability substantially equivalent to that of the original sand prior to use and the addition of said fluoride constituent.

8. A used molding sand for casting magnesium containing about 2 to 5 per cent bentonite, 1 to 2 per cent sulfur, 1 to 2 per cent boric acid, 0.25 to 0.5 per cent potassium fluoride, and about 1.5 to 2.5 per cent of a polyhydric alcohol, said sand being characterized by a flowability substantially equivalent to that of the original sand prior to use and the addition of said fluoride constituent.

ROBERT T. WOOD.